

# UNITED STATES PATENT OFFICE.

WALLACE SAVAGE, OF PIEDMONT, ALABAMA.

## PROCESS OF DETINNING.

1,113,491.

No Drawing.

Application filed February 17, 1914. Serial No. 819,285.

Specification of Letters Patent. Patented Oct. 13, 1914.

To all whom it may concern:

Be it known that I, WALLACE SAVAGE, a citizen of the United States, residing at Piedmont, in the county of Calhoun and 5 State of Alabama, have invented certain new and useful Improvements in Processes of Detinning, of which the following is a specification.

This invention relates to processes of detinning and has particular reference to a 10 process adapted to readily, economically and substantially completely remove tin from tin coated metals and to separately recover the coating and the coated metals.

15 I have discovered that a coating of ordinary white tin may be changed to a dark amorphous non-adherent powder known as gray tin by the catalytic action of gray tin and that the change takes place most satisfactorily 20 when gray tin is employed in connection with a solution of a tin salt, preferably tin ammonium chlorid,  $\text{SnCl}_3\text{NH}_4\text{Cl}$ , which is commonly known as "pink salt." The reaction occurs at ordinary atmospheric temperatures 25 preferably however, below a temperature of 68° F. and somewhat more readily at a temperature of about 32° F. I have found that practical commercial results can be obtained even at a temperature somewhat 30 above 68° F., although a lower temperature is preferred.

In using gray tin to transform white tin into gray tin, it may be applied to the white tin surface in a moist condition or prefer- 35 ably in the form of a slime. I prefer however to employ the gray tin in a solution of a slime. This slime may be advantageously produced by dissolving ten pounds of tin 40 ammonium chlorid in 100 gallons of water and mixing with this solution about 2500 pounds of gray tin.

The slime may be advantageously stirred or otherwise agitated while being used in 45 the detinning operation but I have found

that satisfactory results are obtained by merely moving the material to be detinned into and out of, or preferably through, the slime.

As the white tin is transformed into the 50 gray tin it separates from the metal in the form of a dark amorphous powder having a specific gravity of 5.2.

A part of the gray tin produced in the 55 operation of the process is employed as a catalyst in the detinning operation. The balance is transformed into white tin by melting.

While I have described in detail the preferred operation of my process it is to be understood that the proportions of the re- 60 agents and the temperatures may be varied within wide limit without departing from the spirit of my invention or the scope of the subjoined claims. 65

Having described my invention, I claim:—

1. The process of detinning which consists in subjecting a coating of white tin to the 70 action of a slime containing gray tin, whereby the white tin coating is transformed into gray tin.

2. The process of detinning which consists in subjecting a coating of white tin to the action of a slime containing a solution of a 73 tin salt and a gray tin.

3. The process of detinning which consists in subjecting a coating of white tin to the action of a slime containing a solution of a 80 basic halogen tin compound and gray tin.

4. The process of detinning which consists in subjecting a coating of white tin to the action of a slime containing tin ammonium chlorid and gray tin.

In testimony whereof I affix my signature 85 in presence of two witnesses.

WALLACE SAVAGE.

Witnesses:

JAMES L. CRAWFORD,  
C. L. PARKER.